

## UNITED STATES PATENT OFFICE

2,007,585

BUILDING MATERIAL AND METHOD OF  
MAKING THE SAME

Teikichi Satow, Tokyo, Japan

No Drawing. Application August 22, 1930, Serial  
No. 477,189

5 Claims. (Cl. 106—38)

This invention relates to building materials of a new and useful composition and to a method of making the same.

The object of the invention is to provide building material such as wall boards, floor coverings, tiles, wood carpets or like substances, which are readily and economically manufactured and of great strength and durability.

A further object of the invention includes the use of vegetable proteidal substances such as soy bean meal, castor seed meal, sesame meal, linseed meal and the like, as a binding base either with or without other adhesive as glues, casein, starches and the like, and with said binding base I use a filler of cheap waste material such as hog fuel, sugar cane bagasse, straw chips, hay, wood chips or similar materials properly prepared. In some cases the addition of coarse sawdust or cork waste may be admixed with the above named fillers.

Another object is the use of long fibre fillers so arranged and united that the product produced is very strong and will not bend or warp.

My improved process moreover contemplates the use of a quick setting binding base with a high water resistance as, for example, the vegetable proteidal base and adhesives named above.

A further object embraces the production of a product which will partake of a surface polish and will display the fibres within, which fibres may be further given a marked distinction by the addition of pigments.

Other objects of the invention will appear hereinafter.

The main features of this invention, however, are in the manufacture of building materials from cheap sources such as hog fuel and similar cellulose like materials, which are united with a plastic proteidal binding base such as soy bean binder and shaped or formed under high pressure and dried.

The waste material used preferably includes hog fuel which is a waste wood product of lumber mills and veneer plants and is prepared by disintegrating or grinding in a mill into small pieces.

These pieces constitute the fibrous filler material and vary in size from sawdust to about two or three inches in length. The source of soft wood fibrous materials is very great and, therefore, I will define my invention with respect to said material. It is understood, however, that the use of wood chips, sugar cane bagasse, straw, wheat bran (or equivalents), long wood chips with or without sawdust, long wood chips with or without cork dust and any other long fibre materials are included as fillers. The process, therefore,

includes the use of a cheap fibrous filler thoroughly mixed with a quick setting proteidal binding base and pressed or shaped to the desired form or article, which is then dried and, if desired, machined or polished. As a specific application of the invention I utilize the cellulose fibres of hog fuel thoroughly mixed with a soy bean plastic as the binding base and pressed under high pressure in molds. The soy bean plastic has strong adhesive properties and is used as one component of the plastic to bind the materials together. It, therefore, constitutes a plastic component of a quick setting binding base as will appear more fully hereinafter.

In this invention I use a quick setting binding base with high water resistance. This is important because the binding base is used as a plastic rather than an adhesive. Heretofore the ordinary binding adhesives in the veneer industry were long setting and were made for that purpose as a quick setting adhesive could not be used and would be detrimental to the veneer industry because of, (a) its rapid coagulation, (b) failure of the transfer of adhesive on the core to the outer surface of the dry panel, (c) spoil the adhesive. But in this invention I use the adhesive for plastic purposes, instead of veneering the panel, and, therefore, it is necessary and desirable that a quick setting adhesive be used. The benefits of quick setting adhesives are apparent, as time is saved in the manufacture of the product due to the fact that the products do not have to be under a press for such a long time. Moreover, quick setting plastic adhesives produce strong tenacious final products, which, in the case of wall boards, will not warp or bend. In fact, for the particular purposes of my present invention, the quicker the setting of the binding base the better.

The product obtained by my new process is superior in that it is waterproof and will remain straight in drying. That is it will not curve, bend or warp. This characteristic is believed to be due to the use of the long and short cellulose fibres or wood chips, which act as a reinforcement in every direction throughout the whole mass and, therefore, will not admit of warping. No readjustment of the materials thus made is necessary.

In carrying out my invention I use as the basic substance or filler prepared hog fuel, sugar cane bagasse, straw chips or any similar or equivalent cellulose substance, which is properly ground up so as to furnish the fibrous materials for the filler. These substances either alone or inter-

5

10

15

20

25

30

35

40

45

50

55

mixed are further intimately united with a binding base of suitable vegetable proteidal substances such as soy bean meal, castor seed meal, sesame or linseed meal and the like, taken either alone or mixed together with or without starches, glues, albumens and the like. If desired any color or stain may be given to the products by the addition of pigments or stains added to the basic filler materials.

10 As a specific example the following illustrations are given:

*Example I.*—Take 300 to 400 parts by weight of dry hog fuel or dry wood chips or similar or equivalent basic substance and mix the total mass thoroughly in a mixer with a binding base so that the surfaces of the fibrous materials are thoroughly covered with the binding material.

A suitable quick-setting binding material or base is made as follows:

20 Take 100 parts by weight of soy bean meal, or its equivalent, and add three parts of blood albumen, 10 to 15 parts of lime, 1.5 parts of copper sulfate, 1 part of potassium dichromate and mix them well. Then add 300 parts of water 25 and mix for several minutes. Next add 6 to 10 parts of caustic soda dissolved in 15 parts of water. Mix this for fifteen minutes and then add 30 to 50 parts of silicate of soda and mix for three minutes, and then 10 to 15 parts of a waterproofing liquid may be added.

30 The above named binding material and filler material are thoroughly mixed and the total mass is placed in a suitable mold or equivalent and subjected to a pressure of about 200 to 300 pounds per square inch for several hours (from three hours to overnight). Ordinary room temperature may be used, but if higher temperature is used the setting will be proportionately quicker. After pressing the product for a suitable period 40 of time it is taken out of the molds and dried in air for one or more days as may be determined by actual conditions. The resultant board, tile or other kind of product is thus obtained without the objection of it being warped, curved or 45 crooked while drying. As a final finish the surface may be polished, machined or sanded and a product obtained which is unique in design and beautiful in appearance as well as useful for various purposes where similar manufactured articles are used.

50 The following outstanding characteristics are properties of the products thus produced:

I.—The product so produced is hard and can be substituted in place of hardwood by the use of 55 soft wood base which is much cheaper than the hardwood material. The product will not show any marks by placing heavy furniture, such as a piano, on the finished board or floor.

II.—The product is highly resistant to the action of water. It may be dipped in water for 60 several days without any destructive results and when dried will retain its original hardness.

III.—The product is an excellent heat insulating and sound absorbing material. It may, therefore, be used also as a wall board for concrete and cement buildings as well as for other purposes.

IV.—Its cheapness of commercial production makes the product suitable for wall boards, tiles, 65 floor coverings, wood carpets or the equivalent.

*Example II.*—Use of sugar cane bagasse: Take

500 parts by weight of sugar cane bagasse and mix the same with the binding medium in the proportions given under Example I and after the sugar cane bagasse is thoroughly mixed with the pasty plastic binding material it is pressed in a suitable mold under 200 pounds per square inch for two or more hours. It is then dried as in the case of the wood chips. This gives an excellent sound proofing board.

*Example III.*—Hog fuel or wood chips and other materials: Take a mixture of 200 parts by weight of hog fuel or wood chips and 200 parts of coarse sawdust or 100 parts of coarse cork grain. Mix this thoroughly with the pasty plastic binding medium as explained under Example I 15 and press the total mass under a pressure of 200 to 500 pounds per square inch for a period of two to three hours. Dry the resultant product and, if desired, finish by polishing as before. The cork used in this product will give it a superior elasticity over the product obtained under Example I.

20 It is obvious that various other combinations with the several basic fibre fillers and the proteidal plastic binder as a principal component 25 might be given to illustrate the invention and it should be understood that my invention in its broadest scope as defined in the claims is not to be limited to any specific materials or combinations thereof.

30 What I claim as new and useful and desire to secure by United States Letters Patent is:

1. As an article of manufacture, a building material in the form of a board, tile or floor covering containing the long fibre fillers of comminuted hog fuel and a quick setting vegetable proteidal binding base with a high water resistance and characterized by its hardness of texture and the structural arrangement of the hog fuel in that the wood pieces thereof are disposed in 49 different directions to thereby reinforce each other and resist warping.

2. A building material of the class described derived from long and short cellulose fibre waste comminuted hog fuel combined with a glutenized 45 soy bean meal and having the long and short cellulose fibres disposed to act as reinforcements and thereby prevent warping.

3. The method of making building materials, tiles, floor coverings, and the like which comprises mixing three to four parts of dry comminuted hog fuel with one part of soy bean meal binder and three parts of water containing caustic soda and soda silicate in solution.

4. A composition for building boards, tiles, floor 55 coverings, and like products consisting of three to four parts of fibrous fillers from comminuted hog fuel with one part of soy bean meal binder and three parts of water containing caustic soda and sodium silicate in solution, the fillers arranged and united to produce a strong non-bending, non-warping building product.

5. A composition for building boards, tiles, floor coverings, and like products consisting of three to four parts of fibrous fillers from comminuted 65 hog fuel with one part of soy bean meal binder and three parts of water containing caustic soda and sodium silicate in solution, the fillers arranged to partake of a surface polish for displaying the fibres therein.

70 TEIKICHI SATOW.